

No. 781,458.

PATENTED JUNE 23, 1903.

S. HUGHES & W. F. TAYLOR.  
PACKING.  
APPLICATION FILED AUG. 6, 1902.

NO MODEL.



WITNESSES  
C. Nottingham  
G. J. Downing.

INVENTORS  
S. Hughes and  
W. F. Taylor  
By H. G. Seymour Attorney.

## UNITED STATES PATENT OFFICE.

SAMUEL HUGHES, OF SUMMERTON, AND WILLIAM F. TAYLOR, OF CHARLESTON, SOUTH CAROLINA.

## PACKING.

SPECIFICATION forming part of Letters Patent No. 731,458, dated June 23, 1903.

Application filed August 6, 1902. Serial No. 118,664. (No model.)

*To all whom it may concern:*

Be it known that we, SAMUEL HUGHES, of Summerville, county of Dorchester, and WILLIAM F. TAYLOR, of Charleston, county of 5 Charleston, State of South Carolina, have invented certain new and useful Improvements in Packing; and we do hereby declare the following to be a full, clear, and exact description of the invention, such as will enable others 10 skilled in the art to which it appertains to make and use the same.

Our invention relates to an improvement in packing, the object of the invention being to provide an improved packing which will 15 absorb and retain a large quantity of lubricant, the latter being used to saturate the separate strands before forming the packing, and, further, to provide a packing in which the primary strands are wound about with a 20 wire or fiber and the core-strands not wound, but made soft and pliable to permit the primary strands to sink therein and shape the packing as desired.

With these objects in view the invention 25 consists in certain novel features of construction and combinations and arrangements of parts, as will be more fully hereinafter described, and pointed out in the claims.

In the accompanying drawings, Figure 1 is 30 a view in section, illustrating our improvements in course of construction; Fig. 2, a similar view after compression into shape. Fig. 3 is a view in section of the finished packing. Fig. 4 is a view in elevation, and Figs. 35 5 and 6 are views of a modification.

Our improved packing comprises a series of preferably eight primary strands 1 and core-strands 2. In the smaller sizes of packing, such as shown in Figs. 1, 2, 3, and 4, but 40 four corner-cores 2 are provided, the packing being braided square in the ordinary way around the cores. In the larger forms of packing, such as shown in Figs. 5 and 6, a central core-strand 3 is provided in addition 45 to the corner core-strands 2.

The strands 1 are composed of one or more hemp or other fiber strands first treated with a lubricant, preferably oil and graphite, and braided together to form the strands 1. These 50 strands 1 are wrapped with fine wire 4 or fiber, while the core-strands 2 and 3 are not wrapped at all and are preferably composed of asbestos or other fiber saturated with lubricant

and are soft to yield to the primary strands 1 and permit the packing to shape itself as 55 desired. It will thus be seen that our improved packing consists of four or more soft core-strands saturated with lubricant and braided around with preferably eight primary strands wrapped with fine wire or fiber, 60 the individual strands comprising the primary strands being treated with lubricant before formed into the primary strands, thus resulting in a packing which will contain a large amount of lubricant and owing to the 65 unwrapped cores so shape itself to the machinery as to accomplish the greatest possible usefulness.

A great many changes might be made in the general form and arrangement of the several parts described without departing from our invention, and hence we would have it understood that we do not limit ourselves to the precise construction set forth, but consider ourselves at liberty to make such slight 75 changes and alterations as fairly fall within the spirit and scope of our invention.

Having fully described our invention, what we claim as new, and desire to secure by Letters Patent, is—

1. A packing comprising core-strands saturated with lubricant, and primary strands braided around the core-strands and also saturated with lubricant, said primary strands only individually wrapped with a suitable 85 protecting-strand.

2. A packing comprising core-strands saturated with lubricant, primary strands composed of one or more strands treated with lubricant before forming, and said primary 90 strands braided around the core-strands and wire wrapping on the primary strands only.

3. The method of making packing, consisting in saturating core-strands with lubricant, saturating primary strands with lubricant, 95 wrapping each of said primary strands with wire and braiding said core-strands with the primary strands.

In testimony whereof we have signed this specification in the presence of two subscribing witnesses.

SAM'L. HUGHES.

WILLIAM F. TAYLOR.

Witnesses:

HORATIO C. HUGHES,  
JNO. P. DE VEAUX.